

No. 724,353.

PATENTED MAR. 31, 1903.

A. WALDER & J. T. SCHAFER.  
METHOD OF CASTING CYLINDERS.  
APPLICATION FILED MAR. 27, 1901.

NO MODEL.

2 SHEETS—SHEET 1.

Fig. 1.



5

Fig. 2.



Fig. 3.



Witnesses

C. G. Cramell.

J. R. Selden.

Inventors:

Amos Walder and  
John T. Schaffer,  
By Geo. B. Selden,  
Attorney

No. 724,353.

PATENTED MAR. 31, 1903.

A. WALDER & J. T. SCHAFER.  
METHOD OF CASTING CYLINDERS.

APPLICATION FILED MAR. 27, 1901.

2 SHEETS—SHEET 2.

NO MODEL.



Witnesses

C. G. Gramell

H. R. Selden.

Inventors

Amos Walder and  
John T. Schaffer.  
By Geo. B. Selden,  
Attorney

# UNITED STATES PATENT OFFICE.

AMOS WALDER AND JOHN T. SCHAFER, OF ROCHESTER, NEW YORK,  
ASSIGNORS OF ONE-THIRD TO JOHN O. BREWSTER, OF ROCHESTER,  
NEW YORK.

## METHOD OF CASTING CYLINDERS.

SPECIFICATION forming part of Letters Patent No. 724,353, dated March 31, 1903.

Application filed March 27, 1901. Serial No. 53,076. (No model.)

*To all whom it may concern:*

Be it known that we, AMOS WALDER and JOHN T. SCHAFER, citizens of the United States, residing at Rochester, in the county 5 of Monroe, in the State of New York, have jointly invented an Improved Method of Casting Cylinders, of which the following is a specification, reference being had to the accompanying drawings.

10 Our invention relates to improvements in cylinders having lateral arms, trunnions, or other projections, such as are used for hydraulic presses, riveters, and many other purposes; and our invention consists in so casting 15 the arms, trunnions, or other projections on the cylinder that a sound casting may be produced free from porous or spongy defects or blow-holes.

To more fully describe our invention, reference is had to the accompanying drawings, in which like letters of reference are applied to the same parts in the several views.

Figure 1 is a side view of our improved cylinder, partly in section. Figs. 2 and 3 25 represent the shell detached. Fig. 4 is an end elevation of a cylinder for a hydraulic press, partly in section; and Fig. 5 is a section of the shell on the line 5 5 of Figs. 2 and 3.

A is a hollow cylindrical shell of suitable 30 metal, provided with the hollow boss D at its outer end, to which the pipe conveying the pressure fluid to the interior of the cylinder is attached.

To the shell A, suitably located in respect 35 to the casting B, hereinafter described, is secured a projecting plate K, supported by or attached to the exterior surface of the shell and separated therefrom in any suitable manner, such as by means of the studs J.

40 Surrounding the shell A is a casting B, provided with a laterally-projecting arm C, and the projecting plate H on the shell A is so disposed in relation to the casting B that it is located opposite the lateral arm C of the 45 same, so that when the casting B is cast around the shell A the molten metal completely envelops the plate and, becoming set, is firmly embedded between the plate and shell, thereby securely uniting the parts to-

gether and producing a cylinder-casting without defects and greatly strengthened at the junction of the arm C with the body of the casting. 50

We prefer to cast the plate and studs with the shell A, so that they are all integrally of 55 the same metal; but it is obvious that the plate may be supported in any other suitable way. The plate may be straight or curved, as desired, and it may be of any suitable size relative to the dimensions of the arm C, and 60 in order further to facilitate the incorporation of the metal of the plate with the metal of the casting B we provide the plate with one or more perforations K, so that the metal of the casting B when in its molten state 65 fills up these perforations and more perfectly unites the plate with the casting when finally set. In the drawings we have represented the plate in suitable relative arrangement and with perforations substantially 70 such as we have used successfully in casting cylinders for forty-inch hydraulic presses, in which, as there are two projecting arms C C', we employ the two plates H H'. The shell may be bored or otherwise fitted for the 75 ram or plunger before or after the cylinder is cast around it.

E represents a projecting base or foot plate to support the cylinder, and F F are openings in the arms for the frame of the press. 80

In the production of our improved cylinder we first cast the hollow shell A of suitable size, which is placed in the mold in which the casting B, with its arm or projection C, is subsequently cast. Ordinarily in this operation it is found that the metal is porous or full of blow-holes at the junction of the arm with the body or that the shell becomes defective opposite the arm, and it is therefore difficult to obtain sound castings, and for the 85 express purpose of obviating this trouble we form on or attach to the outer surface of the shell A, opposite the inner end of the arm C of the casting B, the projecting plate H, as above described, so as to allow the molten 90 metal to run into the space I between the plate and the shell for firmly uniting the shell, 95 plate, and casting.

The mold is preferably arranged so that the shell A stands in a vertical position at the time of casting the cylinder B around it.

Thus it will be seen that by our invention we secure with certainty sound cylinder-castings of the largest sizes and adapted for all purposes to which such cylinders can be applied. Our invention is also applicable to casting cylinders of metal other than cast-  
iron.

Having thus described our invention, what we claim, and desire to secure by Letters Patent of the United States, is—

1. A cylinder comprising a shell provided with projecting plates formed integral with but separated therefrom, and a casting constituting an arm or trunnion surrounding said shell and projecting into the space formed between said shell and projecting plates, for more perfectly uniting together the casting, shell and projecting plates.

2. A cylinder comprising a shell provided with a longitudinally-disposed projecting plate secured to but separated therefrom, and a casting constituting an arm or trunnion surrounding said shell and uniting the same with the projecting plate between the shell proper and the projecting plate.

3. A cylinder comprising a shell provided with a plurality of projecting plates secured to but separated therefrom, and a casting surrounding said shell and provided with lateral arms located opposite said projecting plates, a portion of said casting engaging said shell beneath said projecting plates for perfecting the joinder of the shell and casting at the point opposite the lateral arms.

4. A cylinder comprising a shell provided with a plurality of perforated projecting plates secured to but separated therefrom, and a casting surrounding said shell and provided with lateral arms located opposite said projecting plates, a portion of said casting engaging said projecting plates and shell in the space formed between the shell and projecting plates, for more perfectly uniting together the shell and casting.

5. The herein-described method of preventing flaws in the casting of cylinders having one or more projecting arms or trunnions, which consists in placing in a suitable mold a shell having one or more projecting plates attached thereto registering with the proposed position of said arms, with a passage for the molten metal between said plates and the shell, and in subsequently filling the mold with the molten metal, substantially as and for the purposes described.

6. The method of preventing flaws in the casting of heavy metallic bodies provided with laterally-projecting arms, which consists in placing in a suitable mold a metallic mass having one or more projecting plates attached thereto registering with the proposed position of said arms, with passages for the molten metal between said plates and said mass, and subsequently filling the mold with molten metal, substantially as described.

AMOS WALDER.  
JOHN T. SCHAFFER.

Witnesses:

GEO. B. SELDEN,  
H. R. SELDEN.